# EUROPEAN PATENT SPECIFICATION

(11) **EP 0 117 119 B1**
(45) Date of publication and mention of the grant of the patent: **17.07.1991**
(21) Application number: 84300946.5
(22) Date of filing: 14.02.1984
(51) Int. Cl.: B21D 47/02, B32B 15/01

(54) **Stiffened structural member and method of making**
Verstärktes Bauelement und Verfahren zu dessen Herstellung
Member structurel renforcé et procédé de fabrication

(30) Priority: 14.02.1983 US 466193
(43) Date of publication of application: 29.08.1984
(73) Proprietor: TEXAS INSTRUMENTS INCORPORATED, Dallas Texas 75265 (US)
(72) Inventor: Delagi, Richard G., Sharon Massachusetts (US); Trenkler, George, E. Providence Rhode Island (US); Schwensfeir, Robert J., Jr., Attleboro Massachusetts (US)
(74) Representative: Abbott, David John

(56) References cited:
- EP-A- 0 077 613
- DE-A- 2 315 030
- US-A- 2 990 608
- US-A- 3 377 683
- US-A- 4 483 478

## Description

The field of this invention is that of inflated composite metal members and the invention relates more particularly to structural members made from inflated composite metals and to methods for making such structural members suitable for use in high performance aircraft and the like.

In manufacturing high performance aircraft where it is important for structural members used in the aircraft to have very high strength-to-weight ratios and to display very reliable characteristics so they can be made and used with assurance they will perform as intended, it has been conventional to use riveted structural members to achieve desired stiffness at selected locations while also being free of anomalous stresses or local areas of weakness which are typically associated with conventionally welded structural assemblies. Recently however, very high quality titanium structural members have been provided for use in high performance aircraft by means of superplastic forming processes wherein titanium components of the structural members are joined by diffusion bonding and are then inflated by carefully applied hydraulic pressure while the titanium materials are heated to a temperature at which they display desired superplasticity. It is found that the resulting titanium structural members have accurately-formed stiffened portions to provide the members with desired, high strength-to-weight ratios; that the members are free of anomalous stress areas and areas of weakness at the diffusion bond locations; and that the members are adapted to be made and used with greater versatility than was possible with the previously used riveted structural assemblies. It would be desirable to provide similar structural members formed of high strength aluminum alloys and the like for use in high performance aircraft but the slow and involved processes used in making the improved titanium structural members are not suited for use with high strength aluminum alloys which are characterized by surface oxides impervious to the noted diffusion bonding techniques. On the other hand, the processes typically used in making inflated composite aluminum assemblies for use in heat-exchangers or in honeycomb structures and the like have not been suited for producing accurately-formed high strength structural members which are sufficiently free of anomalous stress areas and the like to be useful in high performance aircraft.

There is described in DE-A-2,315,030 a method of making structural metal panels in which a plurality of narrow sheets of metal having the property of superplasticity are bonded to a first sheet of metal with a stop-weld material disposed in a central region of each narrow sheet, and after bonding to the first sheet the second sheets are superplastically expanded by fluid pressure under controlled conditions of temperature and pressure. Titanium based alloys are mentioned as being suitable for the method.

### Summary of the Invention

It is an object of this invention to provide a novel and improved structural member suitable for use in high performance aircraft and the like; to provide such an improved member which is formed of high strength aluminium alloys; to provide novel and improved methods for making such structural members; and to provide such methods which are particularly adapted for making structural members using high strength aluminium alloys.

According to the present invention there is provided a method for making a structural member having selectively stiffened portions for use in an aircraft or the like comprising the steps of disposing a pattern of bond-preventing material on one face of an aluminium alloy metal layer, covering the pattern with a second aluminium alloy metal layer, passing the metal layers between pressure bonding rolls for roll-bonding the metal layers together to form a composite member while leaving areas between the layers defined by the bond-preventing material free of bonds, and establishing elevated fluid pressure in said bond-free areas to deform portions of at least one of the aluminuim alloy metal layers for forming selectively stiffened portions of the member, characterized in that at least one of the aluminium metal layers comprises a precipitation-hardenable aluminium metal alloy which is plastically-deformable to display at least about 60 percent elongation when heated to a selected temperature, the aluminium alloy metal layers are passed between said pressure bonding rolls at a temperature below said selected temperature for elongating and reducing the thickness of the metal layers to form solid phase metallurgical bonds between the layers to provide the composite member while elongating the pattern of bond-preventing material to a predetermined extent to define precisely selected bond-free interfacial areas between the metal layers, the metal layers are heated to a first temperature below said selected temperature to improve the metallurgical bonds between the layers in the solid phase sufficiently to hermetically seal the metal layers together around said bond-free interfacial areas for substantially eliminating areas of substantial weakness in the bonds between the layers outside of said bond-free areas, the metal layers are further heated to said selected temperature at which at least said one metal layer displays said substantial plastic deformation characteristics, the elevated fluid pressure is established in said bond-free interfacial areas to plastically deform a portion of at least said one metal layer for forming selectively stiffened portions of the member, and the alloy of at least said one metal layer of the member is precipitation hardened.

In an example of this invention, a novel structural member results from use of the process which comprises the steps of disposing a pattern of bond-preventing material on one surface of a layer of precipitation-hardenable aluminum alloy or the like, disposing a corresponding second metal layer preferably but not necessarily of the same alloy and thickness in interfacing relation to the first layer to cover the pattern, and passing the metal layers between a pair of pressure bonding rolls to elongate and reduce the thickness of the metal layers to a precisely predetermined extent sufficient to form at least incipient solid phase metallurgical bonds between the layers while also elongating the pattern of bond-preventing material in an accurately predetermined manner to precisely define selected bond-free areas between the layers. Preferably the bond-preventing materials are adapted to decompose and form a gas when heated to a selected temperature, and the alloys used in the member layers preferably have grain refining means or the like adapting the layer materials to be substantially deformed to elongations of 60% or more or even superplastically deformed when heated to said selected temperature. Preferably, the alloys are selected so that thermomechanical processing can be used to produce selected equiaxial on nonequiaxial grain structures, thus providing for selected axes of material deformation. In a preferred embodiment of the method of this invention wherein the metal layers are formed of aluminum, the interfacing surfaces of the metal layers are mechanically cleaned for removing oxides from the surfaces and the metal layers are heated to a limited degree for a limited period of time to free the layer surfaces from moisture without excessively reforming oxides on the layer surfaces just prior to passing the layers between the pressure bonding rolls. Preferably, at least one layer of another aluminum material is disposed between the precipitation-hardenable metal layers as the layers are interfacially arranged. In that way, forming of the noted solid phase metallurgical bonds is facilitated and enhanced and further improved bond quality is achieved. In accordance with this invention, the metal layers are also heated to improve the solid phase metallurgical bonds between the metal layers for hermetically sealing the layers together around the bond-free areas between the layers and for reducing anomalous stresses and localized areas of weakness in the noted bonds, the layers preferably being heated to a temperature below said selected temperature for improving the bonds without substantially decomposing the bond-preventing materials.

The bonded metal layers are preferably restrained between profile molds or forming dies or the like so that the pattern of bond-preventing material between the layers is precisely aligned with selected profile mold configurations provided by the molds. The metal layers are heated to said selected deformation temperature and a selected gas or other fluid pressure is established in the bond-free areas between the layers for deforming selected portions of the metal layers superplastically or the like into the profile mold configurations for providing accurately-formed stiffening portions of the desired structural member. This heating also serves to further improve the bonds between the metal layers and to substantially eliminate anomalous stress and localized areas of weakness in the bonds. Preferably for example, the metal layers are heated to said selected temperature at a selected rate so that the bond-preventing materials are thermally decomposed to form a gas for establishing said selected fluid pressure and for plastically deforming the metal layers at a selected rate to thin out the layer material while avoiding localized necking down of the layer materials within the deformed portions of the metal layers. In that way the stiffened portions of the members are provided with predetermined strength. Preferably, the metal layer materials are then treated in conventional manner for precipitation-hardening the metal layer materials to improve that strength. In that way, it is found that the structural members are accurately-formed to have improved strength-to-weight ratios, are substantially free of anomalous stresses and localized bond weaknesses, and provide the necessary high strength and performance reliability to be used in manufacture of high performance aircraft and the like.

### Description of the Drawings

Other objects, advantages and details of the novel structural member and methods of this invention appear in the following detailed description of preferred embodiments of the invention, the detailed description referring to the drawings in which:
Fig. 1 is a plan view of the novel structural member provided according to a preferred embodiment of the inventive method;
Fig. 2 is a section view along line 2-2 of Fig. 1;
Fig. 3 is a schematic view diagrammatically illustrating a preferred form of the method of this invention;
Fig. 4 is a plan view of a stage product produced in the method of Fig. 3;
Fig. 5 is a partial section view to enlarged scale along line 5-5 of Fig. 4;
Fig. 6 is a partial section view similar to Fig.5 illustrating a step in the method of this invention;
Fig. 7 is a section view similar to Fig. 5 illustrating another step in forming the structural member of Fig. 1;
Fig. 8 is a section view similar to Fig. 5 illustrating characteristics of the structural member. of Fig. 1;
Fig. 9 is a schematic view similar to Fig. 3 diagrammatically illustrating an alternate embodiment of the method of this invention;
Fig. 10 is a section view similar to Fig. 8 illustrating characteristics of the structural member made using the method of Fig. 9;
Fig. 11 is a schematic view similar to Fig. 3 diagrammatically illustrating another alternate embodiment of the method of this invention;
Fig. 12 is a section view similar to Fig. 10 illustrating characteristics of the structural member formed using the method of Fig. 11; and
Fig. 13 is a graph diagrammatically illustrating characteristics of some members provided by embodiments of this invention.

### Description of Preferred Embodiments

Referring to the drawings, 10 in Figs. 1 and 2 indicates a novel structural member made according to the inventive method which is shown to include layer means 12, 14 of high strength, precipitation-hardened aluminum alloys or the like which have solid phase metallurgical bonds (indicated at 16 in Fig. 2) hermetically sealing portions of the metal layer means together around precisely defined. areas (indicated at 18 in Fig. 2) which are free of such bonds. The bond areas 16 are substantially free of anomalous stresses and areas of localized weakness, and selected portions 20 of the metal layer means are deformed over the bond-free areas to provide selectively stiffened portions of the member which are precisely formed and configured so that the structural member has precisely predetermined strength and stiffness characteristics and the like, whereby the member is adapted for use in high performance aircraft and the like to achieve intended strength-to-weight properties and to meet designed structural strength and stiffness specifications. In the structural member 10 for example, the stiffened portions 20 are arranged to provide selected stiffness across the member while also providing intended strength at areas 20a where the member is to be secured to another member or the like as will be understood. Alternately of course, the structural strength member 10 is provided with any other corresponding pattern of stiffened portions within the scope of this invention.

The structural member 10 is formed using an embodiment of the invention so that the structural member has the desired characteristics as noted above. That is, a layer 12 of a precipitation-hardenable metal alloy is advanced by being fed from a coil 22 or the like and a second metal layer 14, also preferably comprising a precipitation-hardenable metal alloy, is advanced as from a second coil 24, or the like so that surfaces 12.1, 14.1 of the layers are moved into interfacing relation to each other and so that the layers are passed between a pair of pressure bonding rolls 26 as is indicated by the arrows 22a, 24a in Fig. 3.

In preferred embodiments of this invention, the metal layers 12 and 14 are typically but not necessarily of substantially equal thickness and each comprises a precipitation-hardenable aluminum alloy preferably having grain refining means or the like in the alloy adapting the alloy to be plastically deformed to a substantial extent or even to be superplastically deformed when the aluminum alloy is heated to a selected deformation temperature. However, other precipitation-hardenable alloys are also used in the layers 12 and 14 within the scope of this invention. In preferred embodiments of the invention for example, the metal layers 12 and 14 are formed of precipitation-hardenable aluminum alloys having nominal compositions by weight as set forth in Table I below:

In such aluminum alloys, the copper, zinc and zirconium constituents for example are believed to serve as grain refining means for enhancing deformability of the alloys so that, when the alloys have been subjected to thermal-mechanical processing and the like in known manner, the alloys are believed to be capable of elongating plastically or superplastically up to the levels set forth in Table I when heated to deformation temperatures as specified in Table I at selected rates. That is, the alloys are deformable to the indicated extents at low but practical and controllable strain rates without fracture and, even when not subjected to full thermal-mechanical preparation for achieving superplasticity or when deformed at somewhat greater strain rates, are still capable of being substantially deformed to elongations of 60% or better suitable for forming aircraft structural members and the like without experiencing anomalous or unpredictable necking down of the alloy materials to any significant extent in the deformed areas. Accordingly, the metal alloys are adapted to be formed into stiffening shapes by controlled gas or other fluid-pressure inflation with assurance that the resulting stiffened member has predicted and reproducible strength properties.

Preferably the surfaces 12.1 and 14.1 of the metal layers are cleaned for removing bond-deterring greases and the like from the layer surfaces before the metal layers are brought into interfacial relation to each other. In a preferred embodiment of the invention for example, the layer surfaces are mechanically cleaned by wire brush means or the like as is diagrammatically illustrated at 28 in Fig. 3 for mechanically removing oxides from the layer surfaces and, where the metal layers 12 and 14 embody aluminum alloy materials as is preferred, the layer surfaces are preferably heated by infrared lamp means or the like as is diagrammatically indicated at 30 in Fig. 3 for freeing the mechanically cleaned surfaces of the layers from moisture just before the layer sufaces are brought into interfacial relation to each other between the pressure bonding rolls 26. Preferably the layer surfaces are heated to a selected limited temperature for a selected period of time for removing such moisture from the layer surfaces while also avoiding excessive reformation of oxides on the layer surfaces. For example, when aluminum layer materials are used, the layer surfaces 12.1, 14.1 are preferably heated to a surface temperature from about 100°C. to about 150°C. for a period from about 1 to 20 minutes just prior to being advanced between the bonding rolls, a particularly preferred heating being for about 2 minutes at 150° C. In that way the metal layers are better adapted to be metallurgically bonded together as is described below.

One or more patterns 32 of a bond-preventing or stop weld material are disposed on at least one of the metal layer surfaces 12.1 and the other metal layer 14 is then brought into interfacing relation to the layer 12 to cover the pattern. The bond-preventing pattern is precisely located on the layer 12 by use of a mask or the like or by transfer from a paper tape or the like or in any other conventional manner within the scope of this invention. Typically for example, a strip of transfer paper 34 or the like is advanced from a reel 36 to a take-up reel 38 and is guided to pass over the metal layer surface 12.1 by guide rolls 40 so that the bond preventing patterns 32 are transferred from the paper to the layer surface 12.1 as the patterns are pressed against the layer surface by the transfer roll 42 as will be understood. In that way, detailed bond-preventing patterns of any selected configuration are accurately positioned on the metal layer 12. In a preferred process the bond-preventing patterns are formed on the strip surface by silk screening although any other conventional process for forming the pattern is used within the scope of this invention. The metal layers 12 and 14 are then bonded together to form a composite metal sheet 44 while leaving areas between the layers defined by the bond-preventing material free of bonds as is illustrated at 32a in Figs. 4-5.

For example, in the method of this invention, the metal layers 12 and 14 are preferably pressed together between the pressure bonding rolls 26 for elongating and reducing the thicknesses of the metal layers to an extent sufficient to form at least incipient solid phase metallurgical bonds 46 (see Fig. 5) between selected portions of the metal layers and for elongating the pattern 32 of bond-preventing material to define selected interfacial areas 32a (see Figs. 4 and 5) between the layers which are free of such bonds. That is, the layer materials are rolled down using the squeezing rolls 26 to form composite metal sheet 44 incorporating the metal layers 12 and 14 which have been elongated in the direction of rolling and bonded together and incorporating the bond-preventing pattern 32 which has also been elongated in the same direction as indicated at 32a and which is now embedded between the layers 12 and 14 in the composite sheet 44. The reduction in thickness of the metal layers 12 and 14 is made under conditions to bring about formation of solid phase, green, metallurgical bonds between the layers, and the bond-preventing pattern 32 provided on layer 12 is originally dimensioned to allow for controlled elongation of a pattern by the pressure rolls 26 under those solid phase bonding conditions. Preferably for example the metal layers as specified in Table I are pressed together at or near room temperature (up to about 100°C.) and the layers are rolled with the rolls 26 preferably heated to about 100° C. for reducing the layer thicknesses on the order of about 50 to 80% in forming initial solid phase bonds 46 between layers of aluminum alloy materials. See Fig. 5. In that way, the solid phase bonding occurs between the layers 12 and 14 throughout areas of interfacial contact between the layers except at the location defined by elongated bond-preventing pattern 32a. In that regard, it is noted that when the metal layers 12 and 14 are of equal thickness and are formed of the same aluminum alloy material, the layer materials are adapted to be symmetrically elongated for elongating the bond-preventing pattern 32 in a precisely predetermined way so that the bond-free interfacial area 32a between the bonded metal layers has a precisely defined configuration.

The bond-preventing material forming the pattern 32 is selected to withstand the rolling deformation as above described without substantially decomposing or separating under the pressure and temperature conditions encountered during the rolling. Preferably however the bond-preventing material is selected so that it disassociates or decomposes when heated or otherwise raised above a selected, relatively higher temperature for generating a gas. In a preferred embodiment of this invention, the bond-preventing material is adapted to decompose and generate a gas when the material is heated to a temperature corresponding to a suitable or preferred plastic deformation temperature of the materials embodied in the metal layers 12 and 14. Preferably for example, where the metal layer materials 12 and 14 comprise aluminum alloys as set forth in Table I, the bond-preventing material is used in the patterns 32 are selected from the group having compositions as set forth in Table II:

The composite metal sheet 44 is heated to a selected temperature by heating means as diagrammatically illustrated at 45 in Fig. 3 for sintering or improving the initial solid phase bonds 46 so that the bonds hermetically seal the metal layers 12 and 14 together around the bond-free interfacial areas as is diagrammatically illustrated at 46a in Fig. 5. Preferably where the bond-preventing patterns 32a are formed of heat-decomposable materials as described above, the metal layers are sintered at a temperature relatively lower than the decomposition temperature of the bond-preventing materials for improving the bonds 46 without substantially decomposing the bond-preventing material. Preferably for example, where the metal layer materials are selected from Table I and the bond-preventing materials from Table II, the composite metal sheet 44 is heated to a temperature in the range from about 150°C. to about 400°C. for a period from about 1 to 8 hours to complete the bonds 46a and to hermetically seal the metal layers 12 and 14 together completely around the bond-free areas 32a. In that arrangement, the hermetic bonds between the metal layers prevent undesired migration of the bond-preventing materials into the areas which are intended to be fully bonded and prevent gases resulting from decomposition of the bond-preventing materials from working between the layers 12 and 14 to cause bond deterioration as will be understood. The hermetic seal of the bonds also prevents oxide reformation at the bonded aluminum layer surfaces in the bonded areas which could also result in bond deterioration. This is particularly advantageous where the layer material has a significant magnesium constituent tending to result in acicular magnesium oxide formations. In that way, it is assured that the bond-preventing pattern 32a precisely defines the edges of the bond-free areas between the layers for purposes to be described below. Such a hermetic seal is also desirable during use of the member 10 as will be understood. The heating of the composite shape 44 for improving the bonds 46 also serves to substantially reduce or even to substantially eliminate anomalous stresses and localized areas of weakness from the bonds 46 illustrated at 47 and 49 in rig. 5 as is diagrammatically indicated by line 46a in Fig. 6. That is, the bond growth relieves stresses 47 which may have been formed in the bond areas during rolling reduction of the thickness of the layers 12 and 14 and reduces bond artifacts 49 so that the bond interface can even be effectively eliminated between the metal layers, the strength of the bond across the interface then substantially corresponding to the strength of the metal layer materials themselves.

It is believed that where the metal alloys of the layers 12 and 14 incorporate grain refining means or the like for enhancing plastic deformability of the alloy materials, the above-described thermal-mechanical process for forming and improving the solid phase metallurgical bonds 6 also serves to enhance the plastic deformability of the alloy materials. That is, where the aluminum alloy materials as specified in Table I are reduced in thickness on the order of 50 to 80% in forming the solid phase bonds 46 and where the bonded layers are then heated to temperatures in the range from 250°C. to 400°C. for periods from 1 to 8 hours for improving the bonds, it is believed that such treatment enhances the formability of the noted aluminum alloys so that they display greater elongation when subsequently deformed as is described below.

In the method of this invention, the composite metal sheet 44 is preferably cut into sections 44a as indicated by broken lines 48 in Fig. 3 so that each of the separate sections 44a includes at least one of the elongated bond-preventing patterns 32a as shown in Fig. 4 and is adapted for forming an individual structural member 10. The separated sheet section 44a is then further formed by blanking or bending or the like as may be desired and is preferably placed and restrained between profile mold sections 50, 52 or the like as is illustrated in Fig. 7 so that individual profile mold configurations 50a are aligned with corresponding portions of the bond-preventing pattern as is indicated at 32a.1 in Fig. 7. Where the pattern 32a is formed between the solid phase bonded layers 12 and 14 as above described, the bond-free area 32a is precisely defined and is easily aligned with the profile mold configurations as will be understood. The composite metal sheet section 44a is then heated to a selected deformation temperature of the layer material as above described and an elevated fluid pressure is established in the bond-free areas 32a between the layers for deforming or inflating at least one of the layers 12 or 14 into a corresponding profile mold configuration 50a to form precisely defined and shaped stiffened portions 20 of the structural member 10 as is indicated by broken lines 20 in Fig. 8. The elevated fluid pressure is adapted to be established between the metal layers by inserting a needle-like nozzle between the layers 12 and 14 or through one of the layers into the bond-free areas 32a and by introducing an hydraulic pressure in known manner within the scope of this invention. Preferably however, where the bond-preventing materials forming the pattern 32a are heat-decomposable as described above to form a gas, the composite metal sheet section 44a is preferably heated to a metal layer deformation temperature at which decomposition of the bond-preventing material also occurs, thereby to establish the desired elevated gas pressure in situ between the metal layers for deforming or inflating parts of the layers to form the stiffened portions 20 of the member. Such heating for deterioration or inflation of the member layers typically serves to further improve the bond between the metal layers. In preferred embodiments of the invention where the metal layers 12 and 14 are formed of aluminum alloys as set forth in Table I and the bond-preventing materials are heat-decomposable as set forth in Table II, and where the layer materials are to undergo substantial plastic deformation defined as 60% elongation or more of the layer materials, the rate of heating of the sheet sections 44a is preferably regulated to be very slow to assure that the desired degree of elevated fluid pressure is achieved in the bond-free areas 32a to provide very low strain rates for achieving the desired deformation of the layer materials by super-plastic deformation or the like without causing any significant necking down of the layer materials in forming the stiffening sections 20 of the member 10. Alternately, where grain growth in the selected alloy may be a problem, a more rapid heating rate may be used.

The structural member 10 formed as above described is then subjected to conventional precipitation hardening procedures for hardening the metal alloys of the layers 12 and 14 in the member, thereby to achieve desired high strength in the member materials as will be understood. Typically for example, that treatment involves heating the member to solutionizing and aging temperatures in conventional sequence. Preferably for example where the materials of layers 12 and 14 are selected from Table I as described above, the member 10 is heated to a solutionizing temperature in the range from 480°C to 530°C. for about 15 minutes to one hour and is then quenched in water at a temperature not over about 30°C. within about 5 seconds of removal from the heating furnace. Such heating typically provides further improvement in the strength of the bonds between the member layers. The member materials are then aged by heating the water to temperatures in the range for about 120°C. to 190°C. for about 3 to 24 hours. Alternately, the materials are aged for longer periods at room temperature or the like in any conventional manner. As procedures for hardening the noted alloys are well known, they are not further described and it will be understood that the hardening steps are conventional.

An alternate embodiment of the method of this invention is diagrammatically illustrated in Fig. 9 wherein previously described components are identified by corresponding numerals. In that alternate method, the metal layer means 12 and/or 14 also comprise an additional layer 54 of another aluminum alloy, the additional layer material being selected to facilitate forming and maintaining of solid phase metallurgical bonds between the precipitation-hardenable alloys of the layers 12 and 14. The additional layer material 54 is preferably bonded to the precipitation-hardened layers 12 and/or 14 by any conventional hot or cold roll bonding or the like so that the bond interfaces 56 between the layers 54 and the layers of the precipitation-hardenable alloys 12 and 14 are substantially free of stress anomalies or localized areas of weakness. The metal layers 12 and 14 are then cleaned and advanced as shown in Fig. 9 so that the additional metal layer means 54 are brought into interfacing relation to each other at the bonding rolls 26 to be located between the precipitation-hardenable portions of the layers 12 and 14 as the metal layers are squeezed together so that the above-described solid phase metallurgical bonds are formed between the metal layers 54 as illustrated in Fig. 10. The initially bonded member is then adapted to be sintered, inflated and hardened as described above and it is found that the characteristics of the resulting member are even further improved over structural member prepared by the previously described methods. Preferably the additional layer materials have thicknesses of at least about 0.010 inches to permit roll bonding without separation but are otherwise preferably limited to about 10% of the thickness of the layers 12 and/or 14 so that the member 10a is primarily composed of the higher strength precipitation-hardenable alloys of layers 12 and 14. Preferably for example, where the alloys of layers 12 and 14 are selected from the precipitation-hardenable aluminum alloys of Table I, the additional aluminum materials are selected from the materials set forth in Table III as follows:

Structural members produced in that alternate method result in structural members having further improved characteristics as is diagrammatically illustrated in Fig. 13. That is, where the strip materials are bonded together without the regulated moisture-removing step and without the interliner layers as described, the strength of the bonds between the layers tends to improve when the layer materials are sintered, heated for inflation, and solutionized as indicated by curve 57a in Fig. 13. Then the peel strength of the bonded layers decreases as the layer materials are more fully hardened. Better bonds are obtained between the layers as is indicated by curve 57b in Fig. 13 when the regulated moisture-removing preheating step is used in the bonding process as previously described. Again, there is a reduction of bond peel strength as the layer materials are hardened as is diagrammatically illustrated by curve 57b. However, where the additional interliner layer material described with reference to Fig. 9 is used, the strength of the bonds between the layers is not only improved but also tends to be more significantly retained as the precipitation-hardened materials of the layers are aged as is indicated by curve 57c in Fig. 13.

In another alternate embodiment of this invention, as diagrammatically illustrated in Fig. 11, a separate additional layer of material 58 is advanced from a separate pay-out reel 60 to be fed between precipitation-hardenable alloy layers 12 and 14 as shown in Fig. 11 as those hardenable alloy layers are advanced between the pressure bonding rolls 26. As illustrated in Fig. 11, the additional metal layer material is also subjected to cleaning and drying as in the case of the metal layers 12 and 14 previously described and the bond-preventing pattern 32 is formed on either of the interfacing layer surfaces of the layers 12, 14 or 58 as shown in Fig. 11. In this alternate embodiment of the invention, the material of layer 56 is also selected to facilitate forming of the solid phase metallurgical bonds as described above and in preferred embodiments of the invention comprises a material selected from Table III. That is, as is shown in Fig. 12, the solid phase metallurgical bonds 62 in the member 10b are formed between opposite sides of the metal layer 58 and the respective precipitation-hardenable alloy layers 12 and 14. Again the thickness of the metal layer 58 is preferably at least 0.010 inches and comprises less than about 10% of the thickness of the metal layers 12 and 14 for reasons noted above. The alternate process also achieves bond advantages as indicated by curve 57c in Fig. 13.

The present invention will be more readily apparent from a consideration of the following illustrative examples.

### Example 1

Two strips of 1145 Alloy Aluminum each about 0.063 inches thick were scrubbed and wire-brushed for physically removing oxides from surfaces of the strips for forming substantially virgin metal surfaces on the strips. The strip surfaces were promptly heated to a temperature of about 100°C. for 15 minutes for removing moisture from the strip surfaces without excessively reforming oxides on the strip surfaces. The strips were then immediately arranged in interfacing relation and were passed between pressure bonding rolls heated to 100°C. where the strips were squeezed together with about 60% reduction in thickness for roll-bonding strip surfaces together to form a composite metal member having solid phase metallurgical bonds between the metal layers. The composite member was then heated to a temperature of 260°C. for 45 minutes in air for improving the bond between the metal strips. A comparison member was prepared in the same manner except that, after wire brushing, the strip surfaces were held at room temperature (20°C.) for 15 minutes before being roll-bonded together. Using conventional peel strength test procedures, it was found that the strips heated to 100°C. for 15 minutes before bonding as described had bond strengths 2 to 3 times stronger than the bonds in the comparison member.

### Example 2

Two strips of 1145 Alloy Aluminum were roll-bonded together as described in Example 1 except that, after wire brushing, the strip surfaces were held at a temperature of 150°C. for 15 minutes before being roll-bonded together. Here the strips were found to be bonded together with bond strengths 3 to 4 times stronger than the bonds in the comparison member noted in Example 1.

### Example 3

Two strips of 1145 Alloy Aluminum were roll-bonded together as described in Example 1 except that, after wire brushing, the strip surfaces were held at a temperature of 200°C. for 15 minutes before being roll-bonded together. Here the strips were found to be bonded together with bond strengths about 2 times greater than in the noted comparison member. In other examples, where longer bond sintering periods were used for improving bonds after initial roll-bonding, even greater bond strength improvements were achieved.

### Example 4

Two strips of precipitation-hardenable 7075 Alloy Aluminum in T-0 temper condition and each about 0.063 inches thick were scrubbed and wire-brushed for mechanically removing oxides from strip surfaces. A pattern of the epoxy-based bond-preventing material identified at C in Table II was disposed at a selected location on the brushed surface of one of the strips by silk screening and was cured by being heated to 200° C. for 3 minutes. The brushed surfaces were then promptly brought into interfacing relation with the bond-preventing pattern there between and were passed between pressure bonding rolls heated to a temperature of about 100° C. for roll-bonding or pressure-welding the strips together. The strips were elongated and reduced in thickness by 60% to form a composite metal member having solid phase metallurgical bonds between the strips except in a bond-free area between the strips which was precisely defined by the pattern of bond-preventing material as elongated during the roll bonding of the strips. The composite member was heated to a temperature of 260° C. for about one hour to improve the metallurgical bonds between the strips in the solid phase and for reducing anomalous stress areas in the bonded strip materials. At that point, the materials were found to have sufficient bond strength between the metal layers to permit convenient handling. The composite member was then restrained between profile molds having mold configurations aligned with the bond-preventing pattern between the metal layers and was heated to a temperature of 427° C. for 30 minutes, suitable for decomposing the bond-preventing material to form a gas in the bond-free area between the member strips so that portions of the strip materials were selectively deformed or inflated over the bond-free areas to form stiffening portions of the composite member. Alternately those portions of the composite member are adapted to be inflated or deformed after heating to the noted temperature by introducing an elevated fluid pressure into the bond-free area between the strips through an inflating nozzle forced between the strips as will be understood. The precipitation-hardenable member materials were then hardened in conventional manner.

The member was found to be stiff, suitable for use as a structural panel member or the like. The deformed portions of the member were found to be free of significantly necked-down portions so that the material in the deformed portions of the member layers were thinned to a relatively uniform extent.

### Example 5

Two strips of precipitation-hardenable 7075-T-0 Alloy Aluminum were scrubbed and wire-brushed for physically removing oxides from surfaces of the strips. A pattern of bond-preventing material was placed on a wire-brushed surface of one of the strips and cured as described in Example 4. Surfaces of the strips were promptly heated to a temperature of about 150° C. for about 15 minutes for removing moisture from the strips without tending to reform excessive thicknesses of oxides on the brushed strip surfaces. The strips were then roll-bonded together and subjected to heating for improving the bond between the metal layers as described with reference to Example 4. At that point the strip materials were found to be bonded together with substantially stronger bonds than the composite member described in Example 4. The composite member was then inflated and hardened as described in Example 4 and the resulting stiffened composite member was found to have characteristics as described with reference to Example 4.

### Example 6

Two strips of precipitation-hardenable 7075-T-0 Alloy Aluminum were scrubbed and were wire-brushed for physically removing oxides from surfaces of the strips. A pattern of bond-preventing material was placed on a wire-brushed surface of one of the strips and cured as described with reference to Example 4. Surfaces of the strips were heated to a temperature of about 150° C. for about 15 minutes for removing moisture from the strips without tending to reform excessive thicknesses of oxides on the brushed strip surfaces. The strips were then roll-bonded together and subjected to heating, and inflating steps as described in Example 4. The member was then heated to a temperature of 480° C. for 15 minutes, was immediately quenched in water at less than 30° C., and was heated to a temperature of 120° C. for about 24 hours for precipitation-hardening the layer materials of the member. It was noted that the strength of the bond between the member layers was reduced during heating of the composite member for precipitation-hardening of the layer materials. However the member was found to be suitable for use as a structural panel member or the like.

### Example 7

Two strips of commercial grade "Alclad" 7075-T-0 Alloy Aluminum were used in forming an inflated structural member. Each strip comprised a layer of precipitation-hardenable 7075 Alloy Aluminum having a layer of 7072 Alloy Aluminum roll-bonded on each outer surface of the 7075 Alloy layer in known manner so that the bond interfaces between the layers of the strip were free of anomalous areas of stress or bond weakness. The 7075 Alloy material was adapted by reason of its composition and previous thermomechanical processing to be plastically deformed to a substantial extent (80% elongation or more) and each of the strips was 0.063 inches thick, the 7072 Alloy layers each comprising about 2.5 to 5.0% of the total thickness of the strip. The strip materials were scrubbed and the 7072 Alloy surfaces of the strips were wire brushed for physically removing oxides therefrom. A pattern of bond-preventing material as described at C in Table II was placed on one of the brushed strip surfaces and cured as described in Example 4 and surfaces of the strips were heated to 150° C. for about 2 minutes for removing moisture from the strip surfaces without tending to reform excessive oxide layers on the brushed strip surfaces. The strips were then roll-bonded together between pressure bonding rolls heated to 100° C. to be reduced in thickness by 60% for forming a composite metal member having solid phase metallurgical bonds between the strips except in bond-free areas precisely defined between the strips by the now elongated pattern of bond-preventing material. The composite member was heated to a temperature of 260° C. for one hour for improving the solid phase bonds between the member, for hermetically sealing the strips together around the bond-free areas, and for substantially eliminating anomalous stress areas or areas of bond weakness between the strips. The composite member as then restrained between profile molds so that profile configurations provided by the molds were aligned with the bond-free areas between the strips. The composite member was then heated to a temperature of 430° C. for 0.5 hours for thermally-decomposing the bond-preventing material to form a gas and for heating the strip materials to a desired plastic deformation temperature so that the strip materials were deformed into the profile mold configurations by the gas to form desired stiffening portions of the composite member. The composite member was then heated to a solutionizing temperature of 480° C. for 15 minutes, was promptly quenched in water at 30° C. or less, and was heated to an aging temperature of 120° C. for 24 hours for precipitation-hardening the strip materials.

The member as formed was found to be strong and stiff and the deformed portions of the member were substantially uniformly thin and were found to be free of significantly necked-down portions. No anomalous stress areas or areas of significant bond weakness were observed in the member and the member was precisely formed with intended dimensions and structural characteristics suitable for permitting use of the member in aircraft structural strength applications. Very high strength bonds were found to exist between the member layers.

### Example 8

Two strips of Alclad 7075-T-0 Alloy Aluminum as described above were prepared as described above and an additional strip of 1145 Alloy Aluminum having a thickness of about 0.020 inches was similarly wire-brushed and heated for removing moisture as described above. A pattern of bond-preventing material was provided on one surface of the 1145 Alloy Aluminum material and was cured. Surfaces of the 1145 Alloy and the 2 Alclad strips were heated to 150° C. for 2 minutes, the 2 Alclad strips were brought into interfacial relation with respective opposite sides of the additional strip material, and the three strips were roll-bonded together with 60% reduction in strip material thickness to form a composite member as previously described. The member was then subjected to heat treatment and inflating steps and was hardened as previously described with reference to Example 6. Here the member layers were found to be very securely bonded together and the member was found to have desirable characteristics as intended and was suitable for use in aircraft structural strength applications as described above.

### Example 9

Two strips of Alclad 7075-T-0 Alloy Aluminum and an additional strip of 6061 Alloy Aluminum were roll-bonded, heat-treated and inflated and hardened as described with reference to Example 8. The structural member as formed was found to have desirable characteristics as described with reference to Example 8.

### Example 10

Two strips of 2024 Alloy Aluminum and an additional strip of 6061 Alloy Aluminum were roll-bonded, heat-treated and inflated for forming a structural member as described above with reference to Example 7. The inflated member was heated to a solutionizing temperature of 495° C. for 15 minues, was immediately quenched in water at 30° C. or less, and heated to an aging temperature of 190° C. for 12 hours. Again the structural member as formed was found to have desirable characteristics suitable for use in aircraft structural applications as described with reference to Example 8.

### Example 11

Two strips of 6061 Alloy Aluminum were roll-bonded, heat-treated and inflated as described with reference to Example 6 for forming a structural member. The inflated member was heated to a solutionizing temperature of 530° C. for 15 minutes, was immediately quenched in water at 30° C. or less, and was heated to an aging temperature of 160° C. for 18 hours for precipitation-hardening the member materials. Again the structural member as formed was found to have desirable characteristics for use in structural applications in aircraft.

### Example 12

Two strips of 7475 Alloy Aluminum were roll-bonded, heat-treated and inflated as described with reference to Example 6 for forming a structural member. The inflated member was heated to a solutionizing temperature of 495° C. for 15 minutes, was immediately quenched in water at 30° C. or less, and was aged at 120°C. for 3 hours and at 155° C. for 3 hours for precipitation-hardening the member materials. Again the structural member as formed was found to have desirable characteristics suitable for use in aircraft structural applications.

It should be understood that although particular embodiments of this invention have been described above by way of illustrating the invention, this invention includes all modifications and equivalents of the disclosed embodiments falling within the scope of the appended claims.

## Claims

1. A method for making a structural member having selectively stiffened portions for use in an aircraft or the like comprising the steps of disposing a pattern (32) of bond-preventing material on one face (12.1) of an aluminium alloy metal layer (12), covering the pattern with a second aluminium alloy metal layer (14), passing the metal layers between pressure bonding rolls (26) for roll-bonding the metal layers together to form a composite member while leaving areas between the layers defined by the bond-preventing material free of bonds, and establishing elevated fluid pressure in said bond-free areas to deform portions of at least one of the aluminium alloy metal layers for forming selectively stiffened portions of the member, characterized in that at least one of the aluminium metal layers comprises a precipitation-hardenable aluminium metal alloy which is plastically deformable to display at least 60 percent elongation when heated to a selected temperature, the aluminium alloy metal layers are passed between said pressure bonding rolls at a temperature below said selected temperature for elongating and reducing the thickness of the metal layers to form solid phase metallurgical bonds between the layers to provide the composite member while elongating the pattern of bond-preventing material to a predetermined extent to define precisely selected bond-free interfacial areas between the metal layers, the metal layers are heated to a first temperature below said selected temperature to improve the metallurgical bonds between the layers in the solid phase sufficiently to hermetically seal the metal layers together around said bond-free interfacial areas for substantially eliminating areas of substantial weakness in the bonds between the layers outside of said bond-free areas, the metal layers are further heated to said selected temperature at which at least said one metal layer displays said substantial plastic deformation characteristics, the elevated fluid pressure is established in said bond-free interfacial areas to plastically deform a portion of at least said one metal layer for forming selectively stiffened portions of the member, and the alloy of at least said one metal layer of the member is precipitation hardened.

2. A method as set forth in claim 1 further characterized in that said precipitation-hardenable metal alloy is selected from the aluminium alloys having compositions as set forth in Table I.

3. A method as set forth in claim 2 further characterized in that the bond-preventing material is heat-decomposable at said selected temperature for establishing said fluid pressure in said bond-free interfacial areas while at least said one metal layer is plastically deformable, and the bond-preventing material and the metal layers are heated to said selected temperature at a selected rate to ensure that said deformation of the precipitation-hardenable alloy layer occurs substantially free of localized necked-down portions of layers.

4. A method as set forth in claim 2 or 3, further characterized in that at least one of said layers comprises an additional layer (54 or 56) of aluminium material introduced between the metal layers before the metal layers are passed between said pressure bonding rolls for facilitating forming of said solid phase metallurgical bonds between the metal layers.

5. A method as set forth in claim 2, 3 or 4, further characterized in that said bond-preventing material is selected from the group consisting of heat-decomposable gas-generating materials as set forth in Table II to have a decomposition temperature corresponding to said selected temperature at which at least said one metal layer displays at least said 60% elongation:

6. A method as set forth in claim 2 characterized in that each of the metal layers comprises a layer of a precipitation-hardenable aluminium alloy having a constituent adapting the metal alloy for superplastic deformation when heated to said selected temperature and having a composition set forth in Table I, and that the method includes the steps of:-
mechanically cleaning surfaces of the aluminium metal layers as provided to remove oxides therefrom,
disposing the pattern of bond-preventing material on a cleaned surface of one of said aluminium metal layers,
heating the mechanically cleaned surfaces of the metal layer to a temperature below said selected temperature for a selected limited period of time to free cleaned surface thereof of moisture without excessively reforming oxides on the cleaned surfaces of the layers, and
disposing a moisture-freed, cleaned surface of the other metal layer in interfacing relation to said one layer over the pattern, before passing the metal layers between said pressure bonding rolls,
and when establishing the selected elevated fluid pressures in said bond-free interfacial areas restraining the heated metal layers against relative movement along bonded portions thereof and defining desired profile mold configurations over said bond-free interfacial areas to permit the metal layers over said areas to deform so that at least one of said precipitation-hardenable metal alloy layers is plastically deformed into said profile mold.

7. A method as set forth in claim 6 further characterized in providing at least one additional layer of an aluminium material selected from Table I,
mechanically cleaning surfaces of that additional aluminium metal layer to remove oxides therefrom,
disposing said pattern of bond-preventing material on a cleaned surface of one of said aluminium metal layers including a cleaned surface of said additional layer,
heating the mechanically cleaned surfaces of the additional metal layer to a first temperature for a selected limited period of time to free those cleaned surfaces of moisture without excesively reforming oxides thereon, and
disposing the additional layer between the cleaned moisture-free surfaces of said pair of metal layers to be in interfacing relation thereto with the pattern between a pair of said surfaces.

8. A method as set forth in claim 7 wherein the metal layers are heated to a temperature in the range 150 °C to 300 °C for a period of time between 5 to 30 minutes to substantially free the layer means of moisture without excessively reforming oxides on surfaces of the layer means.

9. A method as set forth in claim 7 further characterized in that the bond-preventing material is heat-decomposable at said selected temperature for establishing said elevated fluid pressure in said bond-free interfacial areas and the bond-preventing material and the metal layers are heated to said selected temperature at a selected rate to ensure that said deformation of the metal layers occurs while the layer materials display at least 60% elongation.

## Revendications

1. Procédé de fabrication d'un élément de structure possédant des parties sélectivement raidies, destiné a être utilisé dans un aérodyne ou équivalent, comprenant les phases consistant à disposer un dessin (32) de matière anti-liaison sur une face (12.1) d'une couche métallique (12) en alliage d'aluminium, à recouvrir le dessin d'une deuxième couche métallique (14) en alliage d'aluminium , à faire passer les couches métalliques entre des rouleaux de liaison par pression (26) afin de lier les couches métalliques l'une à l'autre par laminage pour former un élément composite tout en laissant exemptes de liaison les zones comprises entre les couches qui sont délimitées par la matière anti-liaison et à établir une haute pression de fluide dans lesdites zones exemptes de liaison pour déformer des parties d'au moins une des couches métalliques en alliage d'aluminium, afin de former des parties sélectivement raidies dans l'élément, caractérisé en ce qu'au moins une première des couches métalliques à base d'aluminium est faite d'un alliage d'aluminium durcissable par précipitation qui peut subir une déformation plastique de façon à présenter un allongement d'au moins 60 % lorsqu'il est chauffé à une température choisie, on fait passer les couches métalliques en alliage d'aluminium entre lesdits rouleaux de liaison par pression à une température inférieure à ladite température choisie, pour allonger les couches métalliques et réduire leur épaisseur de manière à former des liaisons métallurgiques en phase solide entre les couches, pour réaliser l'élément composite, en même temps qu'on allonge le dessin de matière anti-liaison dans une mesure prédéterminée pour définir entre les couches métalliques des zones d'interface exemptes de liaison choisies avec précision, on chauffe les couches métalliques à une première température inférieure à ladite température choisie pour améliorer les liaisons métallurgiques entre les couches dans la phase solide, dans une mesure suffisante pour sceller les couches métalliques à joint étanche tout autour des zones d'interface exemptes de liaison, afin d'éliminer sensiblement les zones de faiblesse notable dans les liaisons établies entre les couches à l'extérieur desdites zones exemptes de liaison, on chauffe davantage les couches métalliques pour les porter à la température choisie, à laquelle ladite première couche métallique présente lesdites caractéristiques de déformation sensiblement plastique, on établit la haute pression de fluide dans lesdites zones d'interface exemptes de liaison pour soumettre à une déformation plastique une partie d'au moins ladite première couche métallique, afin de former des parties sélectivement raidies dans l'élément, et on soumet l'alliage d'au moins ladite première couche métallique de l'élément à un durcissement par précipitation.

2. Procédé selon la revendication 1, caractérisé en ce que ledit alliage métallique durcissable par précipitation est choisi parmi les alliages d'aluminium possédant les compositions indiquées au tableau I.

3. Procédé selon la revendication 2, caractérisé en outre en ce que la matière anti-liaison se décompose à chaud à ladite température choisie pour établir ladite pression de fluide dans lesdites zones d'interface exemptes de liaison alors qu'au moins ladite première couche métallique est capable de subir la déformation plastique, et on chauffe la matière anti-liaison et les couches métalliques à ladite température choisie à une vitesse choisie pour faire en sorte que ladite déformation de la couche d'alliage durcissable par précipitation se produise pratiquement sang rétraints localisés dans les couches,

4. Procédé selon la revendication 2 ou 3, caractérisé en ce qu'au moins une première desdites couches est constituée par une couche additionnelle (54 ou 56) de matière à base d'aluminium qu'on a introduite entre les couches métalliques avant de faire passer les couches métalliques entre lesdits rouleaux de liaison par pression, pour faciliter la formation desdites liaisons métallurgiques en phase solide entre les couches métalliques,

5. Procédé selon la revendication 2, 3 ou 4, caractérisé en outre en ce que ladite matière anti-liaison est choisie dans le groupe composé des matières qui se décomposent à chaud en dégageant des gaz, qui sont citées au tableau II en tant que matières ayant une température de décomposition qui correspond à ladite température choisie à laquelle au moins ladite première couche métallique présente ledit allongement d'au moins 60 %.

6. Procédé selon la revendication 2, caractérisé en ce que chacune des couches métalliques est constituée par une couche d'alliage d'aluminium durcissable par précipitation, qui constitue un constituant rendant l'alliage métallique apte à la déformation superplastique lorsqu'il est chauffé à ladite température choisie, et qui possède une composition telle que celles citées au tableau I, et en ce que le procédé comprend les phases consistant à :
- nettoyer mécaniquement les surfaces des couches métalliques à base d'aluminium de la façon voulue pour en éliminer les oxydes ;
- disposer le dessin de matière anti-liaison sur une surface nettoyée d'une première desdites couches métalliques à base d'aluminium ;
- chauffer les surfaces nettoyées mécaniquement de la couche métallique à une température inférieure à ladite température choisie, pendant un temps limité choisi pour débarrasser de toute humidité la surface nettoyée de cette couche sans reformation excessive d'oxyde sur les surfaces nettoyées des couches ; et
- disposer une surface nettoyée, débarrassée de son humidité, de l'autre couche métallique dans une position relative d'interface avec ladite première couche, par dessus le dessin, avant de faire passer les couches métalliques entre lesdits rouleaux de liaison par pression,
et, lorsqu'on établit les hautes pressions de fluide choisies dans lesdites zones de l'interface qui sont exemptes de liaison, empêcher les couches métalliques chauffées de subir des déplacements relatifs le long de leurs parties liées, et définir des configurations désirées d'un moule de profil au-dessus desdites zones d'interface exemptes de liaison pour permettre aux couches métalliques qui surmontent lesdites zones de se déformer de telle manière qu'au moins une des couches métalliques en alliage durcissable par précipitation subisse une déformation plastique en se moulant dans ledit moule de profil.

7. Procédé selon la revendication 6, caractérisé en outre en ce qu'on prépare au moins une couche additionnelle d'une matière à base d'aluminium choisie dans le Tableau I ;
- on nettoie mécaniquement les surfaces de cette couche métallique additionnelle à base d'aluminium pour en éliminer les oxydes ;
- on dispose ledit dessin de matière anti-liaison sur une surface nettoyée d'une première desdites couches métalliques à base d'aluminium, qui peut éventuellement être une surface nettoyée de ladite couche additionnelle ;
- on chauffe les surfaces nettoyées mécaniquement de la couche métallique additionnelle à une première température pendant une période limitée choisie pour débarrasser lesdites surfaces nettoyées de toute humidité sans reformation excessive d'oxydes sur ces surfaces ; et
- on dispose la couche additionnelle entre les surfaces nettoyées exemptes d'humidité de ladite paire de couches métalliques de façon qu'elle soit en relation d'interface avec lesdites surfaces, le dessin se trouvant entre ces surfaces,

8. Procédé selon la revendication 7, dans lequel on chauffe les couches métalliques à une température de l'intervalle de 150 à 300°C pendant un temps d'entre 5 et 30 minutes, pour débarrasser sensiblement les couches de toute humidité sans reformation excessive d'oxydes sur les surfaces des couches.

9. Procédé selon la revendication 7, caractérisé en outre en ce que la matière anti-liaison se décompose à chaud à ladite température choisie pour établir ladite haute pression de fluide dans lesdites zones d'interface exemptes de liaison et on chauffe les couches métalliques à ladite température choisie, à la vitesse choisie, pour faire en sorte que ladite déformation des couches métalliques se produise pendant que les matières des couches présentent un allongement d'au moins 60 %.

## Patentansprüche

1. Verfahren zum Herstellen eines Bauteils mit selektiv versteiften Abschnitten für die Verwendung in einem Flugzeug oder dergleichen, enthaltend die Schritte der Anbringung eines Musters (32) aus einem verbindungsverhindernden Material auf einer Fläche (12.1) einer Metallschicht (12) aus einer Aluminiumlegierung, des Bedeckens des Musters mit einer zweiten Metallschicht (14) aus einer Aluminiumlegierung, des Hindurchführens der Metallschichten zwischen Druckverbindungswalzen (26) zum Walzverbinden der Metallschichten miteinander zur Bildung eines Verbundbauteils, während Bereiche zwischen den Schichten, die von dem bindungsverhindernden Material festgelegt sind, frei von Verbindungen gehalten werden, und des Erzeugens eines erhöhten Strömungsmitteldrucks in den verbindungsfreien Bereichen zur Verformung wenigstens einer der Metallschichten aus der Aluminiumlegierung zur Bildung selektiv versteifter Abschnitte des Bauteils, **dadurch gekennzeichnet**, daß wenigstens eine der Aluminiummetallschichten eine durch Ausscheidung härtbare Aluminiummetallegierung enthält, die plastisch so verformbar ist, daß sie bei Erwärmung auf eine ausgewählte Temperatur eine Dehnung von wenigstens 60 % zeigt, daß die Metallschichten aus der Aluminiumlegierung zwischen den zwei Druckverbindungswalzen bei einer Temperatur unterhalb der zur Dehnung ausgewählten Temperatur hindurchgeführt werden und die Dicke der Metallschichten so reduziert wird, daß zwischen den Schichten metallurgische Verbindungen in fester Phase zur Erzeugung des Verbundbauteils entstehen, während das Muster aus bindungsverhinderndem Material um ein vorbestimmtes Maß gedehnt wird, damit genau gewählte bindungsfreie Grenzflächenbereiche zwischen den Metallschichten entstehen, daß die Metallschichten auf eine erste Temperatur unterhalb der ausgewählten Temperatur erhitzt werden, damit die metallurgischen Verbindungen zwischen den Schichten in der festen Phase genügend verbessert werden, um die Metallschichten rund um die verbindungsfreien Grenzflächenbereiche hermetisch gegeneinander abzudichten, damit Bereiche mit beträchtlicher Schwäche in den Verbindungen zwischen den Schichten außerhalb der verbindungsfreien Bereiche im wesentlichen eliminiert werden, daß die Metallschichten weiterhin auf die ausgewählte Temperatur erhitzt werden, bei der wenigstens eine der Metallschichten die beträchtlichen plastischen Verformungseigenschaften zeigt, daß der erhöhte Strömungsmitteldruck in den verbindungsfreien Grenzflächenbereichen erzeugt wird, damit ein Teil wenigstens einer Metallschicht zur Bildung selektiv versteifter Abschnitte des Bauteils plastisch verformt wird, und daß die Legierung wenigstens einer Metallschicht des Bauteils durch Ausscheidung gehärtet wird.

2. Verfahren nach Anspruch 1, **dadurch gekennzeichnet**, daß die durch Ausscheidung härtbare Metallegierung aus den Aluminiumlegierungen ausgewählt ist, die die in der Tabelle I angegebenen Zusammensetzungen haben:

3. Verfahren nach Anspruch 2, **dadurch gekennzeichnet**, daß das verbindungsverhindernde Material bei der ausgewählten Temperatur durch Wärme zersetzbar ist, damit der Strömungsmitteldruck in den verbindungsfreien Grenzflächenbereichen entsteht, während wenigstens eine der Metallschichten plastisch verformt wird, und daß das verbindungsverhindernde Material und die Metallschichten mit einer ausgewählten Geschwindigkeit auf die ausgewählte Temperatur erhitzt werden, damit gewährleistet wird, daß die Verformung der durch Ansfällung härtbaren Legierungsschicht im wesentlichen frei von örtlichen Einschnürungsbereichen der Schichten erfolgt.

4. Verfahren nach Anspruch 2 oder 3, **dadurch gekennzeichnet**, daß wenigstens eine der Schichten eine zusätzliche Schicht (54 oder 56) aus Aluminiummaterial enthält, die zwischen die beiden Metallschichten eingeführt wird, ehe die Metallschichten durch die Druckverbindungswalzen hindurchgeführt werden, damit die Bildung der metallurgischen Verbindungen in der festen Phase zwischen den Metallschichten erleichtert wird.

5. Verfahren nach Anspruch 2, 3 oder 4, **dadurch gekennzeichnet**, daß das verbindungsverhindernde Material aus der Gruppe, die aus wärmezersetzbaren, gaserzeugenden Materialien gemäß der Tabelle II besteht, so ausgewählt ist, daß es eine Zersetzungstemperatur hat, die der ausgewählten Temperatur entspricht, bei der wenigstens eine der Metallschichten die Verlängerung von wenigstens 60 % zeigt:

6. Verfahren nach Anspruch 2, **dadurch gekennzeichnet**, daß jede der Metallschichten eine Schicht aus einer durch Ausfällung härtbaren Aluminiumlegierung enthält, die eine Komponente aufweist, die die Metallegierung für eine superplastische Verformung geeignet macht, wenn sie auf die ausgewählte Temperatur erhitzt wird, wobei sie die in der Tabelle I angegebene Zusammensetzung hat, und daß das Verfahren die folgenden Schritte enthält:
mechanisches Reinigen von Oberflächen der Aluminiummetallschichten zum Entfernen von Oxiden, Anbringen des Musters aus verbindungsverhinderndem Material auf einer gereinigten Oberfläche einer der Aluminiummetallschichten, Erhitzen der mechanisch gereinigten Oberflächen der Metallschicht auf eine Temperatur unterhalb der ausgewählten Temperatur für eine ausgewählte begrenzte Zeitperiode zum Befreien der gereinigten Oberflächen von Feuchtigkeit ohne übermäßige Neubildung von Oxiden auf den gereinigten Flächen der Schichten, und Anbringen einer von Feuchtigkeit befreiten, gereinigten Fläche einer weiteren Metallschicht in angrenzende Beziehung an die eine Schicht über dem Muster vor dem Hindurchführen der Metallschichten zwischen den Druckverbindungswalzen, und beim Erzeugen der ausgewählten erhöhten Strömungsmitteldrücke in den verbindungsfreien Grenzflächenbereichen Festhalten der erhitzten Metallschichten gegen eine relative Bewegung längs ihrer verbundenen Bereiche und Bilden gewünschter Profilformkonfigurationen über den verbindungsfreien Grenzflächenbereichen, damit sich die Metallschichten über diesen Bereichen so verformen können, daß wenigstens eine der durch Ausscheidung härtbaren Metallegierungsschichten in die Profilform plastisch verformt wird.

7. Verfahren nach Anspruch 6, **dadurch gekennzeichnet**, daß wenigstens eine zusätzliche Schicht aus einem Aluminiummaterial, das aus der Tabelle I ausgewählt ist, vorgesehen wird, daß Oberflächen dieser zusätzlichen Aluminiummetallschicht zum Entfernen von Oxiden mechanisch gereinigt werden, daß das Muster aus verbindungsverhinderndem Material auf einer gereinigten Oberfläche einer der Aluminiummetallschichten einschließlich einer gereinigten Oberfläche der zusätzlichen Schicht angebracht wird, daß die mechanisch gereinigten Oberflächen der zusätzlichen Metallschicht auf eine erste Temperatur für eine ausgewählte Zeitperiode erhitzt werden, damit diese gereinigten Oberflächen von Feuchtigkeit befreit werden, ohne daß eine übermäßige Neubildung von Oxiden erfolgt, und daß die zusätzliche Schicht zwischen den gereinigten, feuchtigkeitsfreien Oberflächen der zwei Metallschichten in Grenzflächenbeziehung mit diesen mit dem Muster zwischen zwei der Flächen angeordnet wird.

8. Verfahren nach Anspruch 7, **dadurch gekennzeichnet**, daß die Metallschichten auf eine Temperatur im Bereich von 150°C bis 300°C für eine Zeitperiode zwischen 5 und 30 Minuten erhitzt werden, damit die Schichten ohne wesentliche Neubildung von Oxiden auf den Oberflächen der Schichten von Feuchtigkeit befreit werden.

9. Verfahren nach Anspruch 7, **dadurch gekennzeichnet**, daß das verbindungsverhindernde Material bei der ausgewählten Temperatur durch Wärme zersetzbar ist, damit in den verbindungsfreien Grenzflächenbereichen der erhöhte Strömungsmitteldruck erzeugt wird, und daß das verbindungsverhindernde Material und die Metallschichten auf die ausgewählte Temperatur mit einer ausgewählten Geschwindigkeit erhitzt werden, damit gewährleistet wird, daß die Verformung der Metallschichten erfolgt, während die Schichtmaterialien eine Dehnung von wenigstens 60 % zeigen.
